

## UNITED STATES PATENT OFFICE.

CHARLES MILTON STINE, OF CHESTER, PENNSYLVANIA, ASSIGNOR TO E. I. DU PONT DE NEMOURS POWDER COMPANY, OF WILMINGTON, DELAWARE, A CORPORATION OF NEW JERSEY.

## EXPLOSIVE.

1,143,330.

Specification of Letters Patent. Patented June 15, 1915.

No Drawing.

Application filed December 13, 1913. Serial No. 806,417.

*To all whom it may concern:*

Be it known that I, CHARLES MILTON STINE, of Chester, in the county of Delaware and in the State of Pennsylvania, have 5 invented a certain new and useful Improvement in Explosives, and do hereby declare that the following is a full, clear, and exact description thereof.

The object of my invention or discovery 10 is to provide a new explosive having among other desirable qualities, great power, and to such ends my invention consists in the explosive hereinafter specified.

I have discovered that ivory nut or "vegetable ivory" which is obtained from the seeds of certain tropical palms, when nitrated, forms a powerful explosive in itself. I have also discovered that it forms an admirable ingredient in combination with 20 other ingredients to produce explosive mixtures of great power.

When nitrocellulose is mixed with nitro-glycerin the former dissolves in the latter to a greater or lesser degree, forming a jelly-like mass, the stiffness of which depends upon the quality and amount of the nitrocellulose used. It is well known that such a mixture of nitrocellulose and nitro-glycerin becomes less sensitive to detonation by a commercial 25 detonator as the proportion of nitrocellulose is increased, so that if more than about ten parts of nitrocellulose to ninety parts of nitro-glycerin is used, the mixture becomes too insensitive for use as a practical explosive. If the proportion is greatly increased beyond this point, the mixture can 30 not be exploded at all by a commercial detonator. Nitrated ivory nut, on the other hand, is insoluble in nitro-glycerin and does 35 not form therewith a jelly-like mass, and the resulting mixture does not become insensitive when large proportions of nitrated ivory nut are used. Because of this fact, mixtures of nitrated ivory nut and nitro-glycerin in any proportions can be exploded 40 by a commercial detonator. For example, a mixture containing fifty parts of nitrated ivory nut and fifty parts of nitro-glycerin, or a mixture containing sixty parts of nitrated 45 ivory nut and forty parts of nitro-glycerin, have been found to be easily sus-

ceptible to detonation by a small commercial blasting cap.

While I shall give examples of explosive mixtures embodying the use of ivory nut, it 55 is to be understood that the formulas given are merely examples and that my invention is capable of application to every form of explosive and to a wide variety of compositions and proportions of ingredients. I 60 desire to claim the invention in the broadest possible terms. Among such examples may be mentioned the following: I have found, for example, that nitrated ivory nut may be used in any of the usual dynamite mixtures 65 containing nitro-glycerin and that when so used it adds greatly to the strength of the explosive. As an example I may make an explosive of the following composition.

|                    |      |    |
|--------------------|------|----|
| Nitro-glycerin     | 30%  | 70 |
| Nitrated ivory nut | 10%  |    |
| Sodium nitrate     | 55%  |    |
| Wood meal          | 5%   |    |
|                    | 100% | 75 |

The method of nitrating the ivory nut is the subject of a separate application for patent filed by me July 23, 1913, Serial Number 780,656.

This explosive has a strength much greater than that of a dynamite containing 30% nitro-glycerin but without the nitrated ivory nut.

As another example, I give the following 85 composition:

|                    |      |  |
|--------------------|------|--|
| Nitro-glycerin     | 35%  |  |
| Nitro-cotton       | 1%   |  |
| Nitrated ivory nut | 5%   |  |
| Sodium nitrate     | 52%  |  |
| Wood meal          | 7%   |  |
|                    | 100% |  |

This explosive also is much stronger than 95 a dynamite containing 35% nitro-glycerin and 1% nitro-cotton without the addition of nitrated ivory nut.

Nitrated ivory nut can also be used to advantage in nitro-glycerin explosives which 100 contain organic nitro compounds or any of the ordinary ingredients of dynamite.

I have also discovered that nitrated ivory nut can be used to advantage in explosives which do not contain nitro-glycerin. As an example of this type of explosive the following forms a very powerful explosive.

10 Nitrated ivory nut ----- 60%  
Sodium nitrate ----- 40%  
-----  
100%

15 In explosives of this kind it is of course possible to replace with nitrated ivory nut all or part of the sodium nitrate or other oxygen bearing salts such as potassium nitrate, ammonium nitrate, potassium chlorate, etc.; and other ingredients may be added, such as organic nitro compounds, paraffin oils, etc.

20 While I have given specific examples of the use of nitrated ivory nut in explosives, it is to be understood that my invention is not limited to any particular explosive, but that I desire to claim in the broadest possible manner the use of vegetable ivory and similar hemi and pseudo celluloses in explosives.

25 By the term "explosives", I mean to cover not only explosives in general, but also particularly substances like smokeless powder, blasting explosives, charges for blasting caps, primers, fuses, etc.

30 Copies of this patent may be obtained for five cents each, by addressing the "Commissioner of Patents, Washington, D. C."

I claim:—

1. An explosive containing nitro-glycerin and nitrated ivory nut.
2. A dynamite containing nitrated ivory nut.
3. An explosive containing nitro-glycerin, nitro-cotton and nitrated ivory nut.
4. An explosive containing nitro-glycerin, nitro-cotton, an organic nitro compound and nitrated ivory nut.
5. An explosive containing nitro-glycerin, nitrated ivory nut, nitro-cotton, an organic nitro compound, a combustible absorbent and an inorganic oxidizing agent.
6. An explosive containing nitro-glycerin, nitro-cotton, nitrated ivory nut, an organic nitro compound and an inorganic oxidizing agent.
7. A dynamite containing approximately 50 35 per cent. of nitro-glycerin and 5 per cent. of nitrated ivory nut.
8. A dynamite containing approximately 35 per cent. of nitro-glycerin, 5 per cent. nitrated ivory nut, 1 per cent. nitro-cotton and 55 an inorganic oxidizing agent.

In testimony that I claim the foregoing I have hereunto set my hand.

CHARLES MILTON STINE.

Witnesses:

HENRY W. JONES,  
CLIFFORD E. BLYTHE.